

March 24, 1959

E. L. COLE ET AL

2,879,223

METHOD FOR PRODUCING A LUBRICATING OIL

Filed Sept. 21, 1955



1

2,879,223

**METHOD FOR PRODUCING A LUBRICATING OIL**

Edward L. Cole, Glenham, William E. Skelton, Beacon, and Richard K. Meyers, Wappingers Falls, N.Y., assignors to The Texas Company, New York, N.Y., a corporation of Delaware

Application September 21, 1955, Serial No. 535,626

6 Claims. (Cl. 208—97)

This invention relates to a method of imparting lubricating characteristics to a cycle gas oil extract. More particularly, the invention concerns the process of alkylating and subsequent light hydrorefining of a cycle gas oil solvent extract in order to impart lubricating properties thereto.

The term "cycle gas oil" as used herein designates a material obtained during any cracking process such as thermal cracking and the various catalytic cracking procedures, for instance, fixed bed, moving bed and fluid catalytic cracking operations. In these cracking operations a gas oil stock is subjected to treatment from which several hydrocarbon fractions are obtained. The heavier fraction in many cases can be advantageously recycled to the feed stock thereby producing a more refined product. This heavier fraction which is usually recycled is termed "cycle gas oil." In accordance with the present invention the cycle gas oil obtained from the operation of a fluid catalytic cracking unit is preferred since much higher yields of the cycled material are obtained in this operation.

Cycle gas oil has a high aromatic content and, from an economic standpoint, the aromatics are advantageously removed by solvent extraction prior to the introduction of the material into the feed line. Aromatic removal from the cycle gas oil is brought about usually by countercurrent solvent extraction using solvents such as furfural, phenol, Chlorex (beta,beta'-dichloroethyl ether) and the like. In accordance with the present invention furfural is the preferred solvent from an economic standpoint. The highly aromatic extracts produced are, in the solvent refining of the cycle gas oil, nonlubricating materials.

The alkylation of mineral lubricating oil extracts to improve the characteristics of the oil, notably the viscosity-temperature characteristics, is known in the art. It is also known to employ light hydrogenation to improve the viscosity indices of mineral lubricating oil extracts. There are, however, distinct differences between cycle gas oil extracts and mineral lubricating oil extracts. The main differences lie in the greater aromaticity of the cycle gas oil extract, the higher molecular weight and the higher boiling range of the lubricating oil extract. The present invention is concerned with the improvement of a cycle gas oil extract as distinguished from a mineral lubricating oil extract.

In accordance with the present invention we have found that alkylating and subsequently light hydrorefining a cycle gas oil extract yields a suitable lubricating oil having an exceptionally low solid point and carbon residue with accompanying excellent oxidation stability and an improved viscosity index.

The alkylation of the cycle gas oil extracts is preferably carried out with olefin material within the range of naphtha to gas oil olefins with the resulting conversion of the comparatively light extract to that of a lubricating oil stock. Although the molecular weight is sufficiently increased by the alkylation process, it does not increase the viscosity index sufficiently to produce a valuable lubricating oil. These alkylated stocks do, however, show a sur-

2

prising resistance to oxidation with very low varnish propensities and, when blended with other lubricating oils, served to reduce oxidation and varnishing tendencies of the blend to a great extent. In order to utilize the good features of the alkylated cycle gas oil extract, light hydrorefining was carried out in accordance with the present invention to produce a valuable oil having a surprisingly low solid point, low carbon residue with an improved viscosity index and still retaining the good oxidation resistance and anti-varnish properties of the alkylated extract.

The product of the present invention has characteristics which make it particularly valuable as a lubricant at low temperatures. It is also valuable as a jet engine oil blending component, a hydraulic fluid and an automatic transmission fluid component.

In further explanation of the invention, the solvent extract of a cycle gas oil is alkylated in the presence of a catalyst with olefins or other alkylating materials such as alkylhalides or alcohols ranging in molecular weight from about 100 to 300. Examples of alkylation catalyst useful in accordance with the present invention are the well known Friedel-Crafts catalysts including hydrogen fluoride, boron trifluoride, aluminum chloride, ferric chloride and stannic chloride. Also used as catalysts are phosphorus pentoxide, kieselguhr and sulfuric acid. The preferred alkylation catalyst is hydrogen fluoride on the basis of a superior yield with its use. It has been found that this catalyst (HF) functions best when high ratios, ranging from 0.3 to 0.5, of hydrogen fluoride to hydrocarbon (extract+olefin) are used. When this is done, both yield and product quality were superior. The preferred alkylating materials employed are alpha olefins. A good source of these alpha olefins is a highly olefinic naphtha fraction obtained by reaction of synthesis gas ( $H_2-CO$ ) in the presence of an iron catalyst and subsequently freed of oxygenates by the conventional procedures such as passing the olefinic material over a deoxygenating catalyst, for example, a highly absorptive synthetic hydrous magnesium silicate or alumina at a raised temperature or by adsorption with silica gel at ambient temperatures. The temperature range over which alkylation occurs will vary with the catalyst used. In the preferred method of alkylation, using HF as the catalyst, the broad temperature range is from 10 to 150° F. whereas the preferred range is from 25 to 110° F.

The alkylate formed is thereafter sufficiently hydrogenated with a catalyst selected for effecting saturation of alkylated aromatic rings without appreciable concomitant excessive destructive hydrogenation. Examples of mild hydrogenation catalysts which can be used are as follows:

Various nickel-tungsten sulfide mixtures, molybdenum sulfide, cobalt molydate, molybdena alumina, chromia alumina, supported noble metal catalysts, for example, platinumized charcoal or a catalyst comprising alumina, platinum and a combined halogen. Of the foregoing catalysts the nickel-tungsten sulfides are preferred.

The present invention will be better understood by reference to the accompany drawing wherein the single figure is a flow diagram of the process in accordance with the invention.

In general, two initial procedures were used in mixing the charge materials. The first, hereinafter known as procedure "a," was the mixing of the alkylation catalyst with the aromatic extract and then adding the olefin slowly. The second alternative procedure, hereinafter referred to as procedure "b," involved the mixing of the extract and olefin and thereafter adding the alkylation catalyst slowly. Procedure "a" is preferred as its products exhibit slightly lower varnishing tendencies.

After adding all components, stirring is continued in the alkylation reactor long enough to insure that the

reaction has progressed to equilibrium, usually from about 8 to 24 hours in batch operation although somewhat shorter periods may also be used. The catalyst is then separated and the alkylated oil layer is caustic neutralized and washed. The product is then dried, flash-stabilized by distillation at temperatures from 250 to 350° F. at from 1-2 mm. pressure to yield an alkylate ready to undergo hydrogenation.

For light hydrorefining, the alkylate oil, with or without diluent, such as cyclohexane, and hydrogenation catalyst are charged to an autoclave and the system is flushed with hydrogen to remove air. The autoclave is then pressured cold with hydrogen to a point commensurate with the calculated desired pressure at the operating temperature. The pressure range for this type of light hydrorefining in accordance with this invention is from about 500 to 5000 p.s.i.g. and the hydrogen consumption ranges from about 400 to 1500 cubic feet per barrel of alkylated extract. The autoclave is continuously agitated and heated until the hydrogen take-up as measured by a pressure drop, has ceased. The temperature maintained during the reaction ranges from about 500 to 800° F., however, the preferred range is from 600 to 700° F. Pressure was maintained by the addition of hydrogen from a high pressure source when necessary. The oil is thereafter filtered to remove the catalyst and stabilized at increased temperature and decreased pressure with nitrogen blowing.

The following table shows the alkylation reaction conditions and the characteristics of alkylated furfural extracts of cycle gas oil from a fluid catalytic cracking unit. The material used to alkylate was a highly olefinic naphtha fraction rich in alpha olefins and having a boiling range of 150 to 380° F., obtained by the reaction of synthesis gas ( $H_2-CO$ ) in the presence of an iron catalyst and thereafter freed of oxygenates by the conventional procedure of passing the olefinic material over silica gel at room temperature. The extract material had a specific gravity (60/60° F.) of 1.006 and a boiling range of from about 520 to 650° F. The catalyst used for the alkylation step was hydrogen fluoride.

TABLE I

| Charge                                      | Products from Procedure "a" |        | Products from Procedure "b" |        |
|---------------------------------------------|-----------------------------|--------|-----------------------------|--------|
|                                             | Run 1                       | Run 2  | Run 3                       | Run 4  |
| Extract/Olefin; wt.                         | 1.1                         | 0.28   | 0.28                        | 0.28   |
| Catalyst/Olefin; wt.                        | 0.63                        | 0.51   | 0.51                        | 0.51   |
| Catalyst/Hydrocarbon; wt.                   | 0.30                        | 0.4    | 0.4                         | 0.4    |
| Temperature, °F.                            | 32                          | 25     | 35                          | 105    |
| Yield, wt. percent basis hydrocarbon charge | 37.5                        | 33.8   | 34.2                        | 26     |
| Sp. Gr. 60/60° F.                           | 0.9680                      | 0.9307 | 0.9268                      | 0.9364 |
| SUS Vis. at 210° F.                         | 55.2                        | 68.8   | 78.0                        | 88.7   |
| Solid Point, °F.                            | +6                          | -8     | 0                           | +7     |
| Carbon Res., percent                        | 0.71                        | 0.61   | 0.68                        | 1.15   |
| Viscosity Index                             | -99                         | -19    | -3                          | -2     |

The following table demonstrates the excellent properties of alkylated cycle gas oil extract with respect to resistance to oxidation and low varnish forming tendencies. The particular test used in this case was the Toettcher varnish test which is described in U.S. Patent No. 2,674,577, to Frederic C. McCoy, Bill L. Benge, Edwin C. Knowles, and Charles C. Towne, issued August 6, 1954.

TABLE II

Products of Table I

| Toettcher Varnish Test at 350° F. | Product from Procedure "a" | Product from Procedure "b" |
|-----------------------------------|----------------------------|----------------------------|
|                                   | Run 1                      | Run 4                      |
| Varnish wt., mg.                  | 0.1                        | 1                          |
| Neut. No.                         | 1.0                        | 1.7                        |

It can be seen from the above Table II that these materials are excellent with respect to varnish formation. The material prepared by procedure "b" produces somewhat more varnish and for this reason procedure "a" is preferred. Nevertheless, the materials formed by either procedure show surprisingly low varnishing tendencies.

The low neutralization numbers of these materials after being subjected to the Toettcher varnish test demonstrates their excellence with respect to oxidation stability.

It is apparent from Table I that the alkylated products do not exhibit characteristics which are particularly suited to a useful lubricant base oil. The low V.I., high solid point and carbon residue of alkylated extract are undesirable in a lubricant.

The following table shows the pertinent data concerning the hydrorefining of another alkylated cycle gas oil extract from a fluid catalytic cracking unit. The extract was alkylated with a highly olefinic naphtha fraction rich in alpha olefins and having a boiling range of 150 to 380° F., obtained by the reaction of synthesis gas ( $H_2-CO$ ) in the presence of an iron catalyst and thereafter freed of oxygenates by passing the material over silica gel at room temperature.

TABLE III

|                                 |      |  |
|---------------------------------|------|--|
| Charge to autoclave:            |      |  |
| Oil, ml.                        | 300  |  |
| Cyclohexane, ml.                | 100  |  |
| Nickel-tungsten sulfide, g.     | 60   |  |
| Temp., ° F.                     | 635  |  |
| Pressure, p.s.i.g.              | 3000 |  |
| $H_2$ consumption, cu. ft./bbl. | 800  |  |

|                    | Charge | Stabilized Product |
|--------------------|--------|--------------------|
| Sp. Gr. 60/60° F.  | 0.9326 | .08566             |
| Vis. at 210° F.    | 70.7   | 33.7               |
| Solid Point, °F.   | 0      | -70                |
| Car. Res., percent | 0.71   | 0.008              |
| Viscosity Index    | -15    | 64.5               |

The extremely low solid point and carbon residue coupled with the improved viscosity index of the cycle gas oil extract as shown in Table III make this product a useful lubricant particularly for low temperature lubrication.

Obviously, many modifications and variations of the invention, as hereinbefore set forth, may be made without departing from the spirit and scope thereof and, therefore, only such limitations should be imposed as are indicated in the appended claims.

We claim:

1. A method for producing a lubricating oil characterized by a low carbon residue and low solid point which comprises alkylating a cycle gas oil extract with olefinic material within the molecular weight range of naphtha to gas oil olefins to produce an alkylated extract characterized by a high solid point, a high carbon residue and a low viscosity index, and thereafter subjecting the alkylated extract to hydrorefining at a temperature in the range of from 500 to 800° F. and at a pressure in the range of from 500 to 5000 p.s.i.g.

2. A method as described in claim 1 wherein the cycle gas oil extract is alkylated with alpha olefins within the molecular weight range of naphtha to gas oil olefins.

3. A method as described in claim 1 wherein the cycle gas oil extract is alkylated with a deoxygenated highly olefinic naphtha fraction, rich in alpha olefins, obtained by the reaction of hydrogen with carbon monoxide in the presence of an iron catalyst.

4. A method as described in claim 1 wherein the alkylation is performed in the presence of a hydrogen fluoride catalyst wherein the ratio of catalyst to hydrocarbon is in the range of from 0.3 to 0.5, and the temperature is in the range of from 25 to 110° F.

5. A method as described in claim 1 wherein the hy-

5

drogenation takes place at a temperature of from 600 to 700° F. and at a pressure of from 1500 to 4000 p.s.i.g.  
 6. A method as described in claim 1 wherein the hydrefining is carried out in the presence of a nickel-tungsten sulfide catalyst.

6

|             |                         |                |
|-------------|-------------------------|----------------|
| 2,549,111   | Millendorf et al. ----- | Apr. 17, 1951  |
| 2,673,175   | Stratford -----         | Mar. 23, 1954  |
| 2,707,713   | Mattox -----            | May 3, 1955    |
| 2,734,019   | Miller et al. -----     | Feb. 7, 1956   |
| 5 2,762,853 | Jones et al. -----      | Sept. 11, 1956 |

## References Cited in the file of this patent

## UNITED STATES PATENTS

|           |                     |               |
|-----------|---------------------|---------------|
| 2,141,593 | Clarke et al. ----- | Dec. 27, 1938 |
|-----------|---------------------|---------------|

|         |
|---------|
| 665,008 |
| 665,058 |

## FOREIGN PATENTS

|                     |               |
|---------------------|---------------|
| Great Britain ----- | Jan. 16, 1952 |
| Great Britain ----- | Jan. 16, 1952 |